# EUROPEAN PATENT SPECIFICATION

(11) **EP 2 553 132 B1**
(45) Date of publication and mention of the grant of the patent: **06.05.2015**
(21) Application number: 10712049.5
(22) Date of filing: 29.03.2010
(51) Int. Cl.: C22C 38/02, C22C 38/04, C22C 38/06

(54) **STEEL PRODUCT WITH IMPROVED WEATHERING CHARACTERISTICS IN SALINE ENVIRONMENT**
STAHLPRODUKT MIT VERBESSERTEN WITTERUNGSEIGENSCHAFTEN IN EINER SALZIGEN UMGEBUNG
PRODUIT D'ACIER POSSÉDANT DES CARACTÉRISTIQUES DE TENUE AUX INTEMPÉRIES AMÉLIORÉES DANS UN ENVIRONNEMENT SALIN

(43) Date of publication of application: 06.02.2013
(73) Proprietor: Arcelormittal Investigación y Desarrollo SL, 48910 Sestao, Bizkaia (ES)
(72) Inventor: ANTONISSEN, Joachim, B-9971 Lembeke (BE); DE GRAVE, Eddy, B-9270 Laarne (BE); MEJIA GOMEZ, Julieth, Alexandra, B-9000 Gent (BE)
(74) Representative: Pronovem
(86) International application number: PCT/EP2010/054086
(87) International publication number: WO 2011/120550

(56) References cited:
- EP-A1- 0 952 235
- EP-A1- 0 969 112
- EP-A1- 1 398 390
- WO-A1-03/010351
- JP-A- 2001 262 271

## Description

### Field of the Invention

The present invention is related to steel types and products made thereof, which exhibit an increase in corrosion resistance when exposed to a chlorine-rich environment. These steels are known as weathering steels.

### State of the art

Weathering steels have been studied and documented for some time. The corrosion resistance is caused by a layer of rust that forms on the steel surface when it is exposed to the outside environment. Traditional alloying elements which enhance this type of weathering resistance are Cu, P, Cr and Ni. However, traditional weathering steels haven proven to be ineffective in an environment containing Cl ions, i.e. marine or seaside environments. It was observed that the Cl ions destabilize some of the stable components that form the protective oxide layer. Solutions to this problem have been proposed, mainly in the form of changes in the steel composition. The best results have been achieved so far by applying significantly higher levels of Ni. However, given that a high amount of Ni is needed and taking into account that the price of Ni is a highly critical parameter in the commercial exploitation of steels, this solution is not regarded as ideal, and a need has arisen for an alternative to the Ni-solution.

One solution is described in JP2006118011, in the form of a steel composition comprising C, Al, Si, P, Ni, Cu, N, with Sn and/or Sb added in an amount between 0.03 and 0.5wt% and one or more of Ti, Nb, Mo, W, V, Ca or Mg, with the mass ratio of Ni/Cu smaller than or equal to 0.5. The weathering capability in saline environment is mainly obtained by the presence of Sb and/or Sn, which stabilize the amount of Fe2+ ions when the steel is in a wet and saline environment, by reacting with Fe3+ ions, produced by oxidation of Fe2+. However, the use of Sn and/or Sb is disadvantageous for various reasons :
- both Sn and Sb have a detrimental effect on hot ductility as they decrease the solubility of Cu in austenite at high temperature
- Sb has a detrimental effect on weld toughness
- Sn can not be removed from the steel during refining
- Sb causes a risk of forming Stibine (SbH3) - a toxic and flammable compound.

JP-A-2001 262 271 discloses a high tensile strength steel sheet excellent in adhesion of electroplating and ductility.

### Aims of the invention

The present invention aims to provide a weathering steel with a Ni-content in the same order of magnitude as in traditional weathering steels, and with an increased corrosion resistance in marine or seaside conditions, as well as with excellent mechanical properties.

### Summary of the invention

The invention is related to a steel product as disclosed in the appended claims. The invention is in particular related to a steel product as disclosed in the main independent claim, suitable for use in outdoor environments, in particular in saline conditions. The steel product of the invention may be any type of construction element such as a steel sheet or beam. In particular, the invention is related to a steel composition characterized by the following contents (in wt%) :
- Carbon between 0.03 and 0.2,
- Manganese between 0.5 and 2,
- Copper between 0.2 and 0.4,
- Ti between 0.01 and 0.07,
- Cr between 0.2 and 0.5,
- Nickel between 0.1 and 0.2,
- Niobium between 0.02 and 0.1,
- Nitrogen between 0 and 0.01,
- Sulphur between 0 and 0.01,
- Phosphor between 0 and 0.01,
- Aluminium higher than 0 and maximum 1.5,
- Silicon between 0.25 and 1.5,
the balance being Fe and accidental impurities, and wherein the sum of the Al and Si levels is higher than about 0.85wt%.

According to a preferred embodiment, the following narrower ranges are defined for Cu, Ti, Cr, Ni and Nb (in wt%) :
- Copper between 0.2 and 0.4
- Ti between 0.01 and 0.07,
- Cr between 0.2 and 0.5,
- Nickel between 0.1 and 0.2,
- Niobium between 0.02 and 0.1.

According to the preferred embodiment, the steel product according to the invention comprises no Sn and no Sb.

### Detailed description of the invention

The present invention is related to a steel product of the weathering steel type, i.e. a product exhibiting increased corrosion resistance after having been exposed to the outside environment for a given time.

According to the invention, the steel product is defined by a composition consisting of (in wt%):
- Carbon between 0.03 and 0.2,
- Manganese between 0.5 and 2,
- Copper between 0.2 and 0.4,
- Ti between 0.01 and 0.07
- Cr between 0.2and 0.5,
- Nickel between 0.1 and 0.2,
- Niobium between 0.02 and 0.1,
- Nitrogen between 0 and 0.01,
- Sulphur between 0 and 0.01,
- Phosphor between 0 and 0.01,
- Aluminium higher than 0 and maximum 1.5,
- Silicon between 0.25 and 1.5,
the balance being Fe and accidental impurities, and wherein the sum of the Al and Si levels is higher than 0.85wt%. The word 'between' as used above is to be understood as inclusive of the borders of the range in question.

According to a preferred embodiment, the amounts of Cu, Ti, Cr, Ni and Nb are as follows (in wt%) :
- Copper between 0.2 and 0.4
- Ti between 0.01 and 0.07,
- Cr between 0.2 and 0.5 ,
- Nickel between 0.1 and 0.2,
- Niobium between 0.02 and 0.1,
This embodiment combines good weathering behaviour in saline conditions with excellent mechanical properties, due to the minimum amounts of the abovenamed elements (Cu, Ti, Cr, Ni, Nb).

The present invention reveals that the inventive steel compositions favour the formation of fine grained goethite (α-FeOOH) in the corrosion layer forming on the surface of a steel product having these compositions, due to the specific combined Al and Si content. With 'fine grained goethite' is meant goethite with grain sizes from about 8nm to about 15nm. The formation of such fine grained goethite is beneficial for the stability of the oxide layer in saline conditions.

It is to be noted that the inventive compositions do not necessarily include an addition of significant amounts of Ni, regarded as beneficial for weathering resistance in saline conditions. The inventive compositions do not comprise Sn and Sb above an accidental impurity level. Preferably, the steel product of the invention comprises no Sb or Sn. Elements such as Nb, Ti, Cu, Cr are added for improving the mechanical properties of the steel.

The invention is related to any type of steel product having the composition as claimed, e.g. steel sheets or beams, obtained by any standard steel-making process, e.g. hot-rolled or cold-rolled sheets or beams.

### Examples

Table 1 shows the compositions of 3 test samples S1 to S3 having Al and Si contents within the claimed invention, as well as 2 comparative samples C1 and C2 having Al and Si contents falling outside the claimed ranges and/or wherein the combined Al and Si content is less than 0.85wt%. The samples are outside the subject matter of the appended claims because of the presence of Molybdenum in S1 and the lower levels of Ti, Cu, Ni, Cr and Nb. They are however illustrative of the influence of the combined presence of Al and Si on the goethite formation, and hence on the weathering steel behaviour of products of the invention.

The test samples have been obtained by standard steel processing methods, involving at least a hot rolling step, possibly followed by a cold rolling step. The samples were subjected to a dip-dry test during 60 days, using a 0.05M NaCl solution, in order to test weatherability behaviour in saline conditions. As a result, oxide layers were formed on the samples. The composition of these oxide layers was investigated by Mössbauer spectroscopy, used in particular to measure the relative area of superparamagnetic goethite in the oxide layer. Superparamagnetic goethite has a particle size between 8 and 15nm, as opposed to antiferromagnetic goethite, having particle sizes above 15nm.

Table 2 clearly shows that the combined Al and Si contents according to the present invention give rise to a considerable increase in the relative area of fine-grained goethite in the oxide layer.

**Table 1 : example compositions (in wt%)**

| Sample | C | **Si** | **Al** | P | Mn | S | N | Ti | Mo | Cu | Ni | Cr |
|---|---|---|---|---|---|---|---|---|---|---|---|---|
| S1 | 0.19 | **0.35** | **1.2** | 0.077 | 1.6 | 0.006 | 0.005 | 0.007 | 0.025 | 0.02 | 0.025 | 0.025 |
| S2 | 0.07 | **1** | **0.03** | 0.02 | 0.5 | 0.003 | 0.003 | - | - | 0.3 | - | - |
| S3 | 0.07 | **0.25** | **0.8** | 0.02 | 0.5 | 0.003 | 0.003 | - | - | 0.3 | - | - |
| C1 | 0.07 | **0.25** | **0.4** | 0.02 | 0.5 | 0.003 | 0.003 | - | - | 0.3 | - | - |
| C2 | 0.03 | **0** | **1** | 0.01 | 1.8 | 0.003 | 0.007 | - | - | 0.4 | - | - |

**Table 2:Relative area of superparamagnetic goethite (in %)**

| Sample | % |
|---|---|
| S1 | 51 |
| S2 | 40 |
| S3 | 29 |
| C1 | 15 |
| C3 | 16 |

## Claims

1. A steel product consisting of (in wt%):
- Carbon between 0.03 and 0.2
- Manganese between 0.5 and 2
- Copper between 0.2 and 0.4,
- Titanium between 0.01 and 0.07,
- Chromium between 0.2 and 0.5,
- Nickel between 0.1 and 0.2,
- Niobium between 0.02 and 0.1,
- Nitrogen between 0 and 0.01,
- Sulphur between 0 and 0.01,
- Phosphor between 0 and 0.01,
- Aluminium higher than 0 and maximum 1.5,
- Silicon between 0.25 and 1.5,
the balance being Fe and accidental impurities, and wherein the sum of the Al and Si levels is higher than 0.85wt%.

2. The steel product according to claim 1 , comprising no Sn and no Sb.

3. A steel product according to claim 1 or 2, said product being a sheet or beam.

4. Use of a steel product according to any one of the preceding claims, as a product that exhibits an increase in corrosion resistance when exposed to a chlorine-rich environment.

5. Use of a product according to any one of claims 1 to 3 in saline outdoor conditions.

## Patentansprüche

1. Ein Stahlprodukt, das besteht aus (in Gew.-%):
- Kohlenstoff zwischen 0,03 und 0,2,
- Mangan zwischen 0,5 und 2,
- Kupfer zwischen 0,2 und 0,4,
- Titan zwischen 0,01 und 0,07,
- Chrom zwischen 0,2 und 0,5,
- Nickel zwischen 0,1 und 0,2,
- Niob zwischen 0,02 und 0,1,
- Stickstoff zwischen 0 und 0,01,
- Schwefel zwischen 0 und 0,01,
- Phosphor zwischen 0 und 0,01,
- Aluminium zu mindestens 0 und höchstens 1,5,
- Silicium zwischen 0,25 und 1,5,
wobei der Rest Fe und zufällige Verunreinigungen sind, und wobei die Summe der Al- und Si-Spiegel mehr als 0,85 Gew.-% ist.

2. Das Stahlprodukt nach Anspruch 1, das kein Sn und kein Sb umfasst.

3. Ein Stahlprodukt nach Anspruch 1 oder 2, wobei das besagte Produkt ein Blech oder ein Träger ist.

4. Verwendung eines Stahlprodukts nach irgendeinem der vorstehenden Ansprüche als Produkt, das eine erhöhte Korrosionsbeständigkeit aufweist, wenn es einer chlorreichen Umgebung ausgesetzt wird.

5. Verwendung eines Produkts nach einem der Ansprüche 1 bis 3 unter salzhaltigen Außenbedingungen.

## Revendications

1. Produit en acier constitué de (en % en poids) :
- carbone, entre 0,03 et 0,2
- manganèse, entre 0,5 et 2
- cuivre, entre 0,2 et 0,4,
- titane, entre 0,01 et 0,07,
- chrome, entre 0,2 et 0,5,
- nickel, entre 0,1 et 0,2,
- niobium, entre 0,02 et 0,1,
- azote, entre 0 et 0,01,
- soufre, entre 0 et 0,01,
- phosphore, entre 0 et 0,01,
- aluminium, plus de 0 et au maximum 1,5,
- silicium, entre 0,25 et 1,5,
le reste étant Fe et des impuretés accidentelles, et dans lequel la somme des taux d'Al et de Si est supérieure à 0,85 % en poids.

2. Produit en acier selon la revendication 1, ne comprenant ni Sn ni Sb.

3. Produit en acier selon la revendication 1 ou 2, ledit produit étant une tôle ou une poutre.

4. Utilisation d'un produit en acier selon l'une quelconque des revendications précédentes, en tant que produit qui présente une augmentation de la résistance à la corrosion quand il est exposé à un environnement riche en chlore.

5. Utilisation d'un produit selon l'une quelconque des revendications 1 à 3 dans des conditions extérieures salines.
